

April 5, 1938.

**E. J. MULLEN**

**2,113,058**

## PROCESS FOR ROASTING ORES

Filed Nov. 26, 1937



INVENTOR  
*Edwin J. Mullen*  
BY *Joseph A. Ryan*  
ATTORNEY

## UNITED STATES PATENT OFFICE

2,113,058

## PROCESS FOR ROASTING ORES

Edwin J. Mullen, New Rochelle, N. Y., assignor  
to General Chemical Company, New York, N. Y.,  
a corporation of New York

Application November 26, 1937, Serial No. 176,534

10 Claims.

(Cl. 75—9)

This invention is directed to methods for roasting sulfide ores to desulfurize the same and to produce sulfur dioxide for use in the manufacture of sulfuric acid, or for any other purposes desired. The invention is a development of my co-pending applications Serial Nos. 55,808 and 55,809, filed December 23, 1935.

To a substantial extent, present practice in roasting of sulfides such as pyrites includes use of mechanically operated multiple hearth furnaces, such for example as the well-known MacDougall, Herreshoff and Wedge burners. As distinguished from the bed or hearth roasting operation of these burners, it has been suggested to roast finely divided sulfides while in gaseous suspension. Suspension roasting processes such as shown for example in Burgoyne and Cordy U. S. Patent No. 1,758,188 of May 13, 1930 have been developed largely because of availability in recent years of supplies of sulfides, such as flotation concentrates, sufficiently finely divided to permit roasting by suspension methods.

In the present state of the art of producing sulfur dioxide from sulfides, it may be said that probably the major portion of the sulfur dioxide utilized in the manufacture of sulfur trioxide by the contact process is obtained by roasting what is known as pyrites "smalls". The usual run-of-pile of pyrites smalls has been crushed so that 100% passes about a half inch screen. A substantial portion of an ore of this type is sufficiently finely divided for suspension roasting if separated from the coarser material, although a large portion of the smalls, in many cases the major portion, comprises ore too coarse for suspension roasting by present methods. In the present specification, "smalls" is used in a generic sense to define a run-of-pile ore containing some ore fine enough for suspension roasting and some ore too coarse for suspension roasting. The term "coarse" is used to denote ore of too large particle size for roasting by suspension methods, and "fines" is utilized to designate sulfide ores sufficiently finely divided to permit roasting by suspension methods.

Since smalls usually contain a substantial portion of coarse ore, the smalls have heretofore been roasted as in a multi-hearth roaster. While multi-hearth furnaces such as the Wedge and Herreshoff burners provide effective roasting, use of burners of this type is objectionable principally on account of the low capacity per unit of apparatus per unit of time and because the complicated construction and operation involves substantial initial and maintenance expense. On

the other hand, grinding of smalls by usual grinding operations, prior to roasting, to such degree of subdivision that all of the ore may be roasted in gaseous suspension is not desirable since, as well-known, fine grinding is one of the most expensive operations in metallurgical processes and in many instances grinding costs are prohibitive.

As disclosed in my earlier applications, I have previously found that when coarse ore is introduced into a combustion zone and suddenly subjected to certain temperatures, preferably not less than about 1300° F., the coarse ore particles are converted to a frangible, brittle condition making possible ready breaking down or pulverizing to a degree of fineness such that the particles may be roasted thereafter in suspension. Utilizing the principle of such discovery, I have developed a method which may be employed to marked commercial advantage for roasting ores such as pyrites smalls. The invention aims to provide sulfide smalls roasting methods by which grinding costs may be reduced to a minimum and which may be carried out in simple, rugged apparatus readily constructed and economically maintained.

The nature of the invention and the objects and advantages thereof may be fully understood from consideration of the following description taken in connection with the accompanying drawing illustrating in vertical longitudinal section a burner in which the improved process may be carried out.

Referring to the drawing, 10 designates a burner comprising a steel shell or casing 11 within which is placed the furnace lining 12 constructed of suitable refractory material, such as firebrick and defining a roasting chamber 14 of circular, horizontal cross-section. The upper part of the combustion chamber is closed off by a crown 15 the top side of which forms a drying or preheating hearth 17. The shell 11 projects upwardly beyond crown 15 and carries a steel framework 18 which in turn supports ore feeding and rabbelling mechanism for the drying hearth. The surface of hearth 17 is slightly cone-shaped and slopes downwardly toward the shell of the burner. Lying above the hearth are rabbles arms 19 having downwardly projecting plows 20 pitched to work sulfides gradually toward the circumference of the drying hearth. Arms 19 are rotated by motor 22 through shaft 23 supported in bearings so as to maintain the lower ends of plows 20 spaced with respect to the surface of hearth 17. An ore bin 24, mounted on framework 18, discharges ore onto a platform 25 from which the

5

10

15

20

25

30

35

40

45

50

55

smalls are intermittently dropped to the center of drying hearth 17 by a sweep 27 rotating with shaft 23.

Cut through shell 11 and also through the upper edge of lining 12 is a passage 34 through which smalls are passed from hearth 17 into a conduit 35 thru which the smalls are transferred to hopper 36. On rotation of rabble arms 19, the sulfide ore is gradually fed through opening 34 into conduit 35.

The bottom of the combustion chamber is formed by a cone-shaped hearth or hopper 40, of substantial vertical length, terminating in a cinder discharge opening 42 which may if desired be provided with a gas lock mechanism through which cinder may be discharged without permitting gas to escape from the combustion chamber.

Part of the air needed to effect roasting is drawn into chamber 14 thru ports 45, 46, and 47, each provided with a damper or door 49 by means of which the amount of entering air may be regulated.

Numerical 55 indicates a grinder-burner comprising a steel shell 56 having a suitable refractory lining 57 and forming a preliminary grinding-roasting chamber 58. Furnace 55 is rotatably mounted on bearings 60 and 61 and is driven from shaft 63 through gear 64. One end of furnace 55 is provided with a fixed head 66, supported by framework not shown and arranged in relatively gas-tight relationship with the end of the shell 56. The opposite end of furnace 55 projects through opening 68 in the lower portion of the vertical wall of the combustion chamber 14. Smalls are fed into furnace 55 from hopper 36 through conduit 37 controlled by valve 38.

Surrounding the upper portion of the suspension roaster 10 is a jacket 70 provided with an air inlet pipe 71 equipped with a regulating damper 72. After passing through jacket 70 air flows through line 75 into the inlet side of a blower 76. Provision is made for drawing atmospheric air into pipe 75 by means of an air inlet 77 having a regulating damper 78. Air-line 80 is connected at one end to the outlet side of blower 76 and projects thru fixed head 66 into the grinding and preliminary combustion chamber 58.

A gas main 85 for withdrawing gaseous products of combustion from the burner opens into combustion chamber 14 at a point just below crown 15. Main 85 conducts such gases into a waste heat boiler 87 in which steam drum 89, headers 90, and water tubes 91 may be of standard construction. Gases from combustion chamber 14 are discharged through line 85 into a chamber 94, formed partly by vertical fire-wall 95, in which dust entrained in the gases settles out and collects in hopper 97 preferably provided with an air-lock 98 through which dust may be withdrawn without admitting air to chamber 94. After contacting water tubes 91 the gases pass downwardly through chamber 100 in which further settling out of entrained solid particles is effected. Chamber 100 is likewise similarly provided at the bottom with an air-lock discharge 102. Movement of the gases through the system is largely controlled by a blower, not shown, to the inlet side of which gas-line 103 is connected.

The invention is applicable to the roasting of sulfide ores such as iron pyrites, pyrrhotite, zinc sulfide or arsenopyrite, but for convenience operation of the process will be described in connection with the roasting of iron pyrites smalls.

In the following discussion it may be assumed the ore referred to is a run-of-pile or pyrites "small" ore, 100% passing a half inch screen and containing about 50% coarse ore insufficiently finely divided for suspension roasting, and about 50% fines (e. g. 30 mesh or finer) of such size as to permit roasting in suspension.

A supply of pyrites smalls is maintained in bin 24 by suitable conveyor or elevator, not shown. Before roasting is begun, grinding and preliminary roasting chamber 58 and combustion chamber 14 are preheated to temperatures above the ignition point of the ore to be roasted, as by oil burners inserted through conveniently located work-holes not shown. When the desired degree of preheat is obtained, motor 22 is started, and rabble arms 19 and sweep 27 may be rotated at a rate of say one revolution in two minutes. Smalls run continuously out of bin 24 onto platform 25, and on each revolution of shaft 23 a regulated quantity of ore is swept off the platform to approximately the center of drying hearth 17. During rotation of arms 19, the sulfide smalls are gradually worked across the surface of hearth 17, into passage 34, and thence thru conduit 35 into hopper 36. During movement of the smalls over hearth 17, the fines and the coarse ore are thoroughly dried and may be preheated as a rule to about 250° F. and generally not in excess of about 400-500° F.

When starting up the process, in addition to preheating preliminary grinding and roasting chamber 58 and suspension roasting chamber 14 to temperatures in excess of the ignition temperature of the particular sulfide ore being treated, chamber 58 is preheated to temperatures not less than about 1300° F. As will hereinafter appear, during course of operations the extent of combustion of sulfur in chamber 58 is controlled so that such chamber is maintained at 40 temperatures preferably not less than about 1300° F. Owing to the existence of such temperatures in chamber 58 the coarse ore particles charged thereto are very suddenly subjected to relatively high temperatures. Experience indicates the loosely combined sulfur of the coarse ore is practically instantaneously volatilized on sudden introduction of the coarse ore into the high temperature atmosphere in chamber 58, and on account of such sudden exposure to these 50 temperatures and consequent differential expansion, strains are set up in the coarse ore particles thus disrupting and converting the ore particles to a porous condition. When the coarse ore is introduced suddenly into chamber 58 the resulting differential expansion and rapid volatilization of the loosely combined sulfur appears to exert within the lumps of the coarse ore, explosive forces which open up the ore rendering the particles porous and converting the same 60 to a frangible condition offering very little resistance to crushing. It will be appreciated that this makes possible easier and more economical grinding of the coarse fraction and greatly simplifies the equipment required as compared with 65 apparatus for pulverizing all the raw ore to say 30-35 mesh. The sudden subjection of the ore to the high temperatures referred to should be distinguished from gradual heating of the ore to the temperatures indicated. Treatment herein contemplates sudden subjection of coarse ore heated to temperatures say not more than about 400-500° F., to temperatures of not less than about 1300° F.

The mixed coarse ore and fines preheated to 75

not in excess of about 400-500° F. and collecting in hopper 36 run through conduit 37 into chamber 58, rate of feed of sulfides being controlled by a suitable valve 38. As explained above, when these coarse ore particles are suddenly subjected to temperatures preferably not less than 1300° F., such particles are suddenly disrupted and rendered porous and remarkably frangible. In chamber 58 are suitable grinding media such as steel balls or rods, and on rotation of shell 56, the bed of coarse ore particles is tumbled and the particles subjected to attrition. On account of the exceedingly frangible condition into which the coarse ore particles are converted almost immediately, disintegration of the coarse ore to a particle size suitable for suspension roasting is very rapid.

In the present example approximately half of the air needed to effect oxidation of the total sulfur and the iron of the initial ore is fed into chamber 58 through pipe 80. Appreciable roasting of both fines and coarse ore takes place, such roasting however probably comprising principally oxidation of loosely combined sulfur of both fines and coarse ore. Part or all of the air needed in chamber 58 may be drawn into the system through the inlet 71 in the lower end of air pre-heating jacket 70 surrounding the suspension roasting zone 14. In jacket 70, the air may be preheated, for example to 500-600° F. or higher, and is then forced by fan 76 thru line 80 into chamber 58. Operations with respect to the grinding and preliminary roasting phase of the process are controlled so as to maintain in chamber 58 temperatures of not less than about 1300° F., and passage of a gas current of sufficient velocity to sweep up and carry out of chamber 58 and into suspension roasting chamber 14 those particles which are sufficiently fine, e. g., 30-35 mesh and smaller, to permit roasting in gaseous suspension.

The present improvements relate primarily to suspension roasting and it is the object to effect as much roasting as possible in suspension and thereby make use of the economic advantages of suspension roasting, principally simple apparatus. Hence, the purpose of grinder-burner 55 is only to effect subdivision of coarse ore to suspension roasting particle size, and no particular advantage is to be gained by maintaining temperatures in chamber 58 much in excess of 1300-1400° F. To obtain the best economic advantages, preferably temperatures should not be permitted to appreciably exceed 1550° F., because at higher temperatures fusion (conversion to magnetic  $Fe_3O_4$ ) begins to take place. Fused particles are hard and not readily grindable, and hence formation of appreciable amounts of fused particles defeats the primary purpose (conversion to readily grindable form) of the coarse ore treatment in grinder-burner 55. When proceeding so as to maintain the temperatures described tests show that the coarse ore particles for the most part are so frangible as to be crushable by pressure of the hand, this indicating how little attrition and consumption of power are needed to pulverize the coarse ore. The maintenance of proper temperatures, the extent of sulfur combustion, the rapidity of grinding of the frangible coarse ore, and the velocity of the gas current in chamber 58 may be readily obtained by control of feed of smalls from hopper 36, rate of rotation of shell 56, and temperature and amount of air introduced into chamber 58 through pipe 80. It will be appreciated that by

regulation of blower 76, damper 72 in the pre-heating jacket air inlet pipe 71, and damper 78 in cold air inlet pipe 77, the quantity and temperature of the air entering chamber 58 may be very closely controlled. The result of operation of the preliminary grinding-roasting phase of the process is such as to quickly and cheaply reduce all of the coarse ore particles to suspension roasting particle size and to effect some roasting of all of the ore with consequent production of some sulfur dioxide. No particular economies are to be gained by conducting operations in chamber 58 in any way other than to accomplish these ends.

A substantial operating advantage afforded by the preliminary oxidation taking place in chamber 58 is that since substantial quantities of sulfur are burned in chamber 58 corresponding amounts of heat are generated most of which heat is dissipated by radiation from the walls of the rotating shell 56. This leaves less heat to be generated in the suspension roasting zone with the result that the tendencies to slag up and agglomerate the suspension roasting zone cinder are appreciably reduced.

The velocity of gas movement through chamber 58 and suspension roasting zone 14 are controlled by the blower, not shown, in gas main 103, and the auxiliary blower 76 ahead of the grinder-burner 55. By regulation of these two blowers velocity of gas movement to chamber 58 is controlled so as to be just sufficiently high to sweep out of chamber 58 those ore particles which are fine enough, say 30-35 mesh or finer, for suspension roasting. Such gas current containing the fines in suspension is discharged from the outlet end of grinder-burner 55 into the fines roasting zone 14, and on account of the upward movement of gas currents the fines particles travel initially vertically toward the top of combustion chamber 14. In some instances it may be desirable to introduce under positive pressure through one or more injectors 73 a small part of the air to be charged into chamber 14. Such air would aid in carrying the fines particles to the top of chamber 14.

The reason for limiting the amount of air entering chamber 58 is to facilitate maintenance therein of temperatures only sufficiently high to bring about the described relative "explosion" of the coarse ore particles, and not to effect any further combustion of sulfur than is necessary for this purpose. In the present example, using the particular ore comprising about 50% coarse ore and 50% fines, roughly about half of the total amount of air required to combust all of the ore is introduced into chamber 58. Hence, further amounts of air or other oxidizing gas are needed to effect roasting, and such air is drawn into the suspension roasting zone 14 through ports 45, 46, 60 and 47. The rate of movement of the upwardly flowing gas stream in chamber 14 is such that the ore particles are carried upwardly well toward the top of chamber 14. However, since the rate of gas movement upwardly through chamber 14 is appreciably less, on account of the relatively large cross-section of chamber 14, than the velocity of the gas stream passing thru chamber 58, the fines particles soon lose their initial momentum and for the most part drop more or less vertically through chamber 14, dotted line 105 on the drawing indicating the general course of a fines particle through chamber 14.

On introduction of the fines into chamber 14 flash roasting of the fines commences and/or

increases with great rapidity, relatively large amounts of heat are generated, and during the upward and downward course of travel of the fines particles through chamber 14 roasting proceeds to completion. Gas temperatures prevailing in chamber 14 are comparable with those existing in known suspension roasting methods, e. g., of the order of 1800-2000° F. In general, the roasting of the fines particles in chamber 14 is similar to that disclosed in my U. S. Patent No. 2,070,236, of February 9, 1937. The resulting iron oxide cinder drops onto hearth 40 and is discharged from the furnace as required.

In the modification illustrated in the drawing, opening 68 into which the outlet end of grinder-burner 55 projects is relatively in the lower end of the suspension roaster. Gas movement in chamber 14 is in an upward direction, the sulfur dioxide gases being withdrawn from the top of the combustion zone. If desired, opening 68 may be adjacent the top of chamber 14 and grinder-burner 55 mounted in a similarly elevated position. In such modified apparatus, air inlets corresponding with ports 45, 46, and 49 may be located in the upper periphery of the walls of chamber 14 just beneath crown 15. Sulfur dioxide gas outlet 85 would then be located near the bottom of the combustion chamber. In this modification, the travel of the fines and gas in chamber 14 would be in a downward direction only and the suspension roasting phase would be a co-current operation similar to that shown in Burgoyne et al. patent previously mentioned.

The sulfur dioxide gases produced enter waste heat boiler 87 at temperatures of around 1800-2000° F. Heat is recovered in the form of steam and entrained dust settles out and collects in chambers 94 and 100. The gas stream enters line 103 at temperatures of say 500-600° F., and may be purified if desired for use, e. g. in the manufacture of sulfuric acid by the contact process.

The invention has been described in connection with roasting of smalls containing about 50% coarse ore and 50% fines because the usual run of smalls contains coarse ore and fines in approximately these proportions. It will be understood, however, that the process of the invention is readily adaptable to handle smalls containing less or greater quantities of coarse ore. In the case of smalls containing less amount of coarse ore, the smalls may be fed to grinder-burner 55 at a greater rate, and where the smalls contain greater quantities of coarse ore rate of introduction of smalls may be correspondingly reduced. Regulation of control conditions in accordance with the nature of the smalls used will be apparent to the skilled operator.

The invention presents several substantial operating advantages. For example, when working with pyrites smalls passing a half inch screen as mentioned, it would ordinarily be necessary to roast this type of ore in a multi-hearth burner or go to the expense of grinding the ore to a sufficient degree of fineness to permit roasting by suspension methods. In accordance with the present process, on account of the exceedingly frangible condition to which the coarse ore is rapidly converted, whatever grinding is necessary may be accomplished with much less expenditure of power than would be the case if the coarse ore constituents were pulverized in usual grinding operations. By the present method, smalls may be roasted in a way much more efficient than could be accomplished in a multi-hearth roaster. An outstanding advantage af-

firmed by the invention is that operations may be carried out in simply constructed and economically maintained apparatus.

I claim:

1. The method for roasting coarse metal sulfide ore which comprises maintaining a zone at temperatures not less than about 1300° F., introducing the coarse ore into said zone whereby the ore is suddenly subjected to temperatures of the combustion zone and converted to a relatively porous frangible condition, subjecting the ore while in said zone to attrition sufficient to reduce the coarse ore to fines, then introducing said fines into a combustion zone, forming therein a suspension of fines in oxidizing gas, roasting the fines while in suspension in the oxidizing gas to produce sulfur dioxide, and recovering sulfur dioxide.

2. The method for roasting coarse metal sulfide ore which comprises maintaining an oxygen-containing combustion zone at temperatures not less than about 1300° F., introducing the coarse ore into said zone whereby the ore is suddenly subjected to temperatures of the combustion zone, converted to a relatively porous frangible condition and partially roasted, subjecting the ore while in said zone to attrition sufficient to reduce the ore to fines, then introducing said fines into a second combustion zone, forming therein a suspension of fines in oxidizing gas, roasting the fines while in suspension in the oxidizing gas to produce sulfur dioxide, and recovering sulfur dioxide.

3. The method for roasting coarse metal sulfide ore which comprises introducing the coarse ore into an oxygen-containing combustion zone heated to temperatures not less than about 1300° F. whereby the ore is suddenly subjected to temperatures of the combustion zone, converted to a relatively porous frangible condition and partially roasted, maintaining such temperatures by at least partial combustion of some of said ore, subjecting the ore while in said zone to attrition sufficient to reduce the ore to fines, then introducing said fines into a second combustion zone, forming therein a suspension of fines in oxidizing gas, roasting the fines while in suspension in the oxidizing gas to produce sulfur dioxide, and recovering sulfur dioxide.

4. The method for roasting metal sulfide smalls containing coarse sulfide ore and initial sulfide fines which comprises maintaining an oxygen-containing combustion zone at temperatures not less than about 1300° F., introducing the smalls into said zone whereby the smalls are suddenly subjected to temperatures of the combustion zone and the coarse ore is converted to a relatively porous frangible condition and partially roasted, subjecting the coarse ore while in said zone to attrition sufficient to reduce the same to fines, then introducing such resulting fines together with said initial fines into a second combustion zone, forming therein a suspension of fines in oxidizing gas, roasting the fines while in suspension in the oxidizing gas to produce sulfur dioxide, and recovering sulfur dioxide.

5. The method for roasting metal sulfide smalls containing coarse sulfide ore and initial sulfide fines which comprises introducing the smalls into an oxygen-containing combustion zone heated to temperatures not less than about 1300° F. whereby the smalls are suddenly subjected to temperatures of the combustion zone and the coarse ore is converted to a relatively porous frangible condition and partially roasted, main-

5 taining such temperatures by at least partial combustion of some of said smalls, subjecting the coarse ore while in said zone to attrition sufficient to reduce the same to fines, then introducing such resulting fines together with said initial fines into a second combustion zone, forming therein a suspension of fines in oxidizing gas, roasting the fines while in suspension in the oxidizing gas to produce sulfur dioxide, and recovering sulfur dioxide.

10 6. The method for roasting metal sulfide smalls containing coarse sulfide ore and initial sulfide fines which comprises maintaining an oxygen-containing combustion zone at temperatures not less than about 1300° F. and not substantially in excess of about 1550° F., introducing the smalls into said zone whereby the smalls are suddenly subjected to temperatures of the combustion zone and the coarse ore is converted to a relatively porous frangible condition and partially roasted, subjecting the coarse ore while in said zone to attrition sufficient to reduce the same to fines, then introducing such resulting fines together with said initial fines into a second combustion zone, forming therein a suspension of fines in oxidizing gas, roasting the fines while in suspension in the oxidizing gas to produce sulfur dioxide, and recovering sulfur dioxide.

15 7. The method for roasting metal sulfide smalls containing coarse sulfide ore and initial sulfide fines which comprises introducing the smalls into a combustion zone heated to temperatures not less than about 1300° F. whereby the smalls are suddenly subjected to temperatures of the combustion zone and the coarse ore is converted to a relatively porous frangible condition and partially roasted, passing through said zone a gas stream containing oxygen in amount less than that needed to support complete oxidation of said smalls but in quantity sufficient to maintain such temperatures by at least partial combustion of some of said smalls, subjecting the coarse ore while in said zone to attrition sufficient to reduce the same to fines, regulating the velocity of the gas stream passing through said zone so as to sweep out of said zone fines resulting from such attrition together with said initial fines, introducing the gas stream containing such fines into a second combustion zone, forming therein a suspension of fines in oxidizing gas in amount sufficient to effect substantially complete oxidation of said fines, roasting the fines while in suspension in the oxidizing gas to produce sulfur dioxide, and recovering sulfur dioxide.

20 8. The method for roasting metal sulfide smalls containing coarse sulfide ore and initial sulfide fines which comprises introducing the smalls into a combustion zone heated to temperatures not less than about 1300° F. whereby the smalls are suddenly subjected to temperatures of the combustion zone and the coarse ore is converted to a relatively porous frangible condition and partially roasted, passing through said zone a gas stream containing oxygen in amount less than that needed to support complete oxidation of said smalls and in quantity restricted to maintain such temperatures not substantially in excess of about 1550° F., subjecting the coarse ore while in said zone to attrition sufficient to reduce the same to fines, maintaining the velocity of the

25 gas stream passing through said zone high enough but not substantially in excess of that required to sweep out of said zone fines resulting from such attrition together with said initial fines, introducing the gas stream containing such fines into a second combustion zone, forming therein a suspension of fines in oxidizing gas in amount sufficient to effect substantially complete oxidation of said fines, roasting the fines while in suspension in the oxidizing gas to produce sulfur dioxide.

30 9. The method for roasting metal sulfide smalls containing coarse sulfide ore and initial sulfide fines which comprises introducing the smalls into a combustion zone heated to temperatures not less than about 1300° F. whereby the smalls are suddenly subjected to temperatures of the combustion zone and the coarse ore is converted to a relatively porous frangible condition and partially roasted, passing through said zone a gas stream containing oxygen in amount less than that needed to support complete oxidation of said smalls but in quantity sufficient to maintain such temperatures by at least partial combustion of some of said smalls, subjecting the coarse ore while in said zone to attrition sufficient to reduce the same to fines, regulating the velocity of the gas stream passing through said zone so as to sweep out of said zone fines resulting from such attrition together with said initial fines, introducing the gas stream containing such fines into the lower portion of a second combustion zone, forming therein a suspension of fines in an upwardly-moving stream of gas containing oxygen in amount sufficient to effect substantially complete oxidation of said fines, roasting the fines while in suspension in the oxidizing gas to produce sulfur dioxide, and withdrawing sulfur dioxide from the upper end of said second combustion zone.

35 10. The method for roasting metal sulfide smalls containing coarse sulfide ore and initial sulfide fines which comprises introducing the smalls into a combustion zone heated to temperatures not less than about 1300° F. whereby the smalls are suddenly subjected to temperatures of the combustion zone and the coarse ore is converted to a relatively porous frangible condition and partially roasted, passing through said zone a gas stream containing oxygen in amount less than that needed to support complete oxidation of said smalls and in quantity restricted to maintain such temperatures not substantially in excess of about 1550° F., subjecting the coarse ore while in said zone to attrition sufficient to reduce the same to fines, maintaining the velocity of the gas stream passing through said zone high enough but not substantially in excess of that required to sweep out of said zone fines resulting from such attrition together with said initial fines, introducing the gas stream containing such fines into the lower portion of a second combustion zone, forming therein a suspension of fines in an upwardly moving stream of gas containing oxygen in amount sufficient to effect substantially complete oxidation of said fines, roasting the fines while in suspension in the oxidizing gas to produce sulfur dioxide, and withdrawing sulfur dioxide from the upper end of said second combustion zone.

40 70 EDWIN J. MULLEN.